

## UNITED STATES PATENT OFFICE.

FRANCIS GEORGE RAWLING, OF MADISON, WISCONSIN, DEDICATED, BY MESNE ASSIGNMENTS, TO THE CITIZENS OF THE UNITED STATES OF AMERICA.

## METHOD FOR THE PREVENTION OF CORROSION IN STEEL DIGESTERS.

No Drawing.

Application filed March 21, 1925. Serial No. 17,370.

(GRANTED UNDER THE ACT OF MARCH 3, 1883; 22 STAT. L. 625.)

*To all whom it may concern:*

Be it known that I, FRANCIS GEORGE RAWLING, a citizen of the United States of America, and an employee of the Department of Agriculture, residing in the city of Madison, State of Wisconsin, whose post-office address is Madison, Wisconsin, have invented a new and Improved Method for the Prevention of Corrosion in Steel Digesters, of which the following is a specification.

This application is made under the act of March 3, 1883, chapter 143 (22 Stat. 625), and the invention herein described and claimed may be used by the Government of the United States, its officers and employees, and by any person in the United States without the payment to me of any royalty thereon. I hereby dedicate the same to the free use of the Government and the people of the United States.

Hitherto, in the processes of manufacturing paper pulp from wood, by cooking such material with an aqueous solution of sodium sulphite, in steel digesting vessels, a serious amount of corrosion of the steel has developed, in such an amount as to render the digesting vessel useless after a short period of time. As the use of a steel vessel is very desirable, it is necessary to find some means of preventing the corrosion of the steel which takes place during the cooking process. The use of an aqueous solution of caustic soda has been tried, by adding this to the digesting liquid, but owing to the action of caustic soda on the wood, an undesirable quality of pulp is produced. There is also a limit to the amount of caustic soda, which may be added to the digester, as an excess prevents the proper production of pulp from the wood by means of the sodium sulphite.

The use of caustic soda solution is not successful in preventing the corrosion of the steel digesting vessel, when used in such quantity that a pulp is produced having the quality of one made by cooking wood with sodium sulphite alone.

This invention relates to the addition of the sodium salts of a polybasic acid, which is not strongly ionized in solution, to the solution of sodium sulphite used for cooking the wood, with the subsequent addition of caustic soda solution, during the actual

period of cooking. When proper amounts of the sodium salt of the polybasic acid and of caustic soda are used, no free caustic soda is present in the cooking liquor at any time, but the condition of alkalinity of the cooking liquid is sufficiently strong, that the latter does not corrode the steel vessel or digester in which the cooking is done.

According to my present invention, wood is boiled under pressure with an aqueous solution of sodium sulphite, containing the sodium salt of a weakly ionized polybasic acid (for example, sodium carbonate, sodium silicate, sodium borate, sodium phosphate, and others), with the subsequent addition to the digester, during the period of digestion, of an aqueous solution of caustic soda, at such a rate that the digesting solution remains alkaline in reaction, yet does not contain caustic soda in sufficient amount to alter the quality of the resulting pulp, from that of a pulp prepared from wood by means of a sodium sulphite solution.

It is to be understood that the proportion of sodium sulphite to the sodium salt of the weakly ionized polybasic acid may be varied between wide limits and that the caustic soda solution may be added continuously or intermittently to the digester during the period of cooking; also, that the term sodium salt of a weakly ionized polybasic acid is not to be limited to the four salts mentioned, and that one or more of such salts may be used in the same solution of sodium sulphite.

Having thus described my invention in above specification, I desire to secure by Letters Patent the following claims:

1. The process of adding the sodium salt of a weakly ionized polybasic acid to an aqueous solution of sodium sulphite to be used for the pulping of wood, in a steel vessel, with the subsequent addition of a solution of caustic soda to the contents of the steel vessel during the period of cooking, for the purpose of preventing corrosion of the said vessel.

2. The process of adding a mixture of the sodium salts of weakly ionized polybasic acids to an aqueous solution of sodium sulphite, to be used for the pulping of wood, in a steel vessel, with the subsequent addition of a solution of caustic soda to the con-

tents of the steel vessel during the period of cooking, for the purpose of preventing the corrosion of the said vessel.

3. The process of adding sodium carbonate to an aqueous solution of sodium sulphite, to be used for the digesting of wood, in a steel vessel, with the subsequent addition

of a solution of caustic soda to the contents of the steel vessel, during the period of cooking, for the purpose of preventing the corrosion of the said vessel. <sup>10</sup>

December 26th, 1924.

FRANCIS GEORGE RAWLING.